

April 7, 1936.

E. H. BUNCE ET AL

2,036,566

ZINC OXIDE

Filed March 24, 1933



INVENTOR  
Earl H. Bunce  
Harry M. Haslam

BY

Pennie, Davis, Marvin & Edmonds  
ATTORNEYS

## UNITED STATES PATENT OFFICE

2,036,566

## ZINC OXIDE

Earl H. Bunce and Harry M. Haslam, Palmerton, Pa., assignors to The New Jersey Zinc Company, New York, N. Y., a corporation of New Jersey

Application March 24, 1933, Serial No. 662,518

2 Claims. (Cl. 23—148)

This invention relates to the manufacture of zinc oxide and has for its object the provision of certain improvements in zinc oxide manufacture. A particular aim of the invention is the provision 5 of certain improvements in the manufacture of zinc oxide from zinc vapor resulting from the reduction of a porous charge of agglomerates of mixed zinciferous and carbonaceous materials in an upright or vertical reducing chamber.

10 Zinc oxide is commonly made by the oxidation or combustion of metallic zinc vapor. Atmospheric air is the ordinary oxidizing agent, and the resulting fume of zinc oxide particles in suspension in air is drawn or forced through a flue system 15 to a bag-room or other appropriate zinc oxide collecting apparatus, air being thus used for the pneumatic transportation of the zinc oxide particles through the flue system.

It has heretofore been recognized that a certain amount of gas, such as air, exhaust gases, etc. may be introduced with advantage into the residue discharge or lower end of an upright or vertical reducing chamber during the reduction 20 of a porous charge of agglomerates. To this end, the agglomerates are of such a character that they do not break down or disintegrate into fines during the reducing operation, so that gas may be introduced through the residue about to be discharged, either by the suction due to the stack 25 draft of the retort (with the bottom of the retort open) or by injection under pressure (with the bottom of the retort sealed). The main advantage of introducing appropriate amounts of gas into the lower end of the upright reducing chamber 30 is the prevention of loss of zinc in the discharged residue. Zinc vapor tends to diffuse downwards in the retort and condense on the cooling residue about to be discharged. The introduction of gas in amounts sufficient to create an upward gas current of sufficient velocity to 35 counteract this tendency of the zinc vapor to diffuse downwards thus results in keeping the residue free from zinc that would otherwise condense therein and be lost.

40 The amount of gas introduced at the bottom of the reducing chamber must be carefully regulated. If too little gas be introduced, the velocity of the ascending gas current will not be sufficient to prevent the diffusion of zinc vapor into the residue. The introduction of an over-supply of 45 gases containing oxidizing constituents such as air or CO<sub>2</sub> may develop so much heat as to fuse or melt the charge, causing it to run out of the bottom of the reducing chamber. Such fusion of the charge is accompanied by loss of zinc and

injury to the reducing chamber. Even though the charge merely becomes pasty, there results a closing up or diminution of the voids between the agglomerates, thereby lowering the permeability of the charge to gas flow and thus retarding effective reduction. Furthermore, too much gas (even if the gas be neutral or reducing) may result in such an excessive dilution of the zinc vapor evolved from the retort as to have an undesirable effect on the zinc oxide product, notably imparting to it too little hiding power or body for use in paint. A very large excess of oxidizing gases may cause part of the zinc vapor to be burned to zinc oxide in the reducing chamber instead of in the contemplated combustion or oxidation chamber or zone, in which case the zinc oxide may be rendered gritty or discolored by overheating in the retort. The introduction of excess gas at the bottom of the reducing chamber 15 may set up such a strong current of gas 20 through the chamber as to entrain particles of the charge which mingle with the zinc oxide product and render it gritty and specky.

25 In making zinc oxide from zinc vapor derived from the reduction of a porous charge of agglomerates in an upright reducing chamber, we have found that the suction necessary for withdrawing the oxide from the oxidizing or combustion zone and for transporting it to the collecting 30 apparatus exercises a marked effect on the pressure prevailing in the reduction chamber, and therefore on the gas current flowing therethrough. In case the bottom of the retort is open, the effect of such suction is ordinarily to augment or supplement the normal stack-draft effect 35 of the reducing chamber, with consequent increase in the amount of gas entering at the bottom. In case the bottom of the retort is sealed, the effect of such suction is to create a vacuum 40 in the retort that tends to facilitate the inflow of injected gas, and even of combustion gases from the heating chamber surrounding the retort, if the wall of the retort is permeable to gases on account of the presence of cracks. The inflow 45 of such combustion gases exerts a corrosive effect on the retort wall and may enlarge minute cracks to dangerous leaks.

50 We have now discovered that the pressure in the retort and the ascending gas current therein may be controlled, with consequent regulation of the amount of gas introduced at the bottom of the chamber, by appropriately regulating and controlling the effect thereon of the current of air supplied to burn the zinc vapor to zinc oxide and 55

to transport the zinc oxide to the collecting apparatus.

Based on these considerations and discoveries, our present invention, in its broad aspect, involves blowing or otherwise appropriately admitting air in controlled amount into the zinc oxide flue system for promoting the transportation therethrough of the fume. More particularly, the invention involves, in making zinc oxide from zinc vapor resulting from the reduction of a porous charge of agglomerates in an upright reducing chamber, control of the amount of gas introduced into the lower end of the reducing chamber by regulating (1) the air supplied (by blasting or otherwise) for the oxidation of the zinc vapor or (2) the air admitted to the flue system for promoting the pneumatic transportation of the oxide therethrough, or both. In the practice of the invention in its complete aspect, there is a three-fold control of the gas and air supply:

(1) Gas or primary air is introduced at the bottom of the reducing chamber in amounts adequate to prevent condensation of zinc in the residue without injuring the quality of the zinc oxide produced.

(2) Secondary air is supplied to the current of zinc vapor from the reducing chamber to burn it to zinc oxide.

(3) Tertiary air is supplied to the zinc oxide formed in order to facilitate its pneumatic transportation to the bag-room.

Part of the tertiary air may be supplied together with the secondary air at the same inlet or inlets; or all of the tertiary air may be admitted either by blowing or by suction at an inlet or inlets separate from the inlets supplying the secondary air, and located so far from the inlets of the secondary air as not to affect the flame with which the zinc vapor burns to zinc oxide.

Fig. 1 of the accompanying drawing diagrammatically illustrates an apparatus adapted for the practice of the invention, and

Fig. 2 illustrates a modified form of apparatus with which the invention may be practiced.

Referring to the drawing, the reducing chamber is shown as a vertically disposed and externally heated retort 10 surrounded by a heating chamber or laboratory 11 of a furnace structure 12. The upper end of the retort 10 preferably extends a substantial distance above the upper end of the furnace structure and constitutes a prolongation 13 in which purification of the zinc vapor may be carried out as described in United States Patent No. 1,749,127, March 4, 1930, wherefore a relatively pure (lead-free) zinc oxide pigment may be made when desired. The lower end of the retort 10 joins a downwardly extending charge confining member 10a which dips into a liquid-seal 35 that provides a gas-tight discharge for the solid residue. The reduced charge may be regulated in its passage through the retort 10 and the extension 10a by means of a discharge rotor 36. Tuyères 37, attached to appropriate supply pipes not shown, are provided just above the discharge rotor for introducing exhaust gases, steam or primary air, in regulated amounts, into the retort.

An off-take pipe or conduit 14 extends laterally from the top of the retort or its prolongation for the withdrawal of the gaseous products of the reducing operation, principally metallic zinc vapor and carbon monoxide. A charging well 15 is provided within the upper end of the prolongation 13 and extends a short distance below the opening of the off-take pipe 14 thereby avoiding obstruction of the latter by the charge. In the drawing,

the charging well 15 is shown closed by a removable cap 16. When the reducing operation is conducted as a continuous process, the cap 16 is replaced by an appropriate charging device for delivering charge to the retort as required while maintaining the top of the retort closed or sealed for all practical purposes.

The off-take pipe 14 has a vertically disposed zinc vapor outlet 17 in its top wall. A nozzle 18, registering with the outlet 17, is mounted above 10 the outlet and is surrounded by an air or wind-box 19 having an annular slot 20 adjacent to and surrounding the mouth of the nozzle 18.

A pipe 21 supplies compressed air from a blower or air compressor 22 to the interior of the wind-box 19. The pipe 21 is provided with a slide damper 23 for regulating and controlling the air delivered to the wind-box. An off-take flue 24 is operatively mounted above the wind-box 19 for conveying the fume of suspended zinc oxide 20 particles to the bag-room or other zinc oxide collector. A suction fan 25 is included in the flue 24. The flue system comprises the necessary series of flues and suction fans for withdrawing the zinc oxide from the zone of combustion and pneumatically transporting it to the zinc oxide collector.

Air for promoting or for facilitating the transport of the zinc oxide through the flue system is supplied under pressure to the flue 24 by a pipe 26 connected to the blower or compressor 22. The pipe 26 has a slide damper 27 for regulating and controlling the amount of air thus supplied to the flue 24. The pipe 26 communicates with the flue 24 at a point so far removed from the zone 35 of combustion or oxidation as not to affect the flame with which the zinc vapor burns to zinc oxide.

In the operation of the apparatus of Fig. 1, the vertical retort 10 and its prolongation 13 are kept 40 full of the charge of non-disintegrating agglomerates of zinc ore and reduction fuel, fresh agglomerates being introduced through the charging well and spent residues being withdrawn from the bottom of the retort as required. Gas (such 45 as exhaust gas) or primary air is admitted at the bottom of the retort to prevent condensation of zinc in the residue. A circumferential blast of secondary air is directed against the stream of zinc vapor and carbon monoxide issuing from 50 the nozzle 18. The resulting particles of zinc oxide are suspended in the resulting gases (for the most part, carbon dioxide, nitrogen and such excess of air as may be supplied by the blast) and are withdrawn from the zone of combustion 55 or oxidation (at the lower end of the flue 24) by the suction of the fan 25 and transported through the flue system to the bag-room or other collecting apparatus. Tertiary air for promoting the transport of the zinc oxide particles through the flue 60 system is supplied to the flue 24 by the pipe 26.

The amount of gas or primary air entering the bottom of the retort is determined by the following factors:

(1) a In the case of a retort with open bottom, 65 the natural stack-draft of the retort and its appurtenances (determined by its permeability to gases, temperature, and the tendency of the zinc vapor and carbon monoxide evolved therein to set up a back pressure).

(1) b In the case of a retort with closed bottom, 70 the pressure at which gas or primary air is supplied by the tuyères 37 at the bottom of the retort.

- (2) The amount of suction developed by the fan 25.  
 (3) The volume and rate of air introduction through the pipe 21.  
 5 (4) The volume and rate of air introduction through the pipe 26.

The relative amounts of air supplied by the pipes 21 and 26 will be largely determined by the contemplated character of the operation. In 10 general, the greater the amount of air introduced through the pipe 21, and hence directed as a blast against the zinc vapor, the greater will be the dilution and the more sudden the cooling of the resulting zinc oxide particles, and hence the 15 finer or smaller will be the average particle size of the resulting zinc oxide product. The contemplated characteristics of the zinc oxide product will therefore determine in a large measure the amount of air to be supplied for blasting 20 through the pipe 21. Since, in practice, it will ordinarily be desirable to maintain this factor substantially constant during the production of any particular grade of zinc oxide, the control of the amount of gas or primary air admitted at the 25 bottom of the retort will be principally effected by regulation and control of the pressure at the tuyères 37 and of the tertiary air supplied by the pipe 26.

As has hereinbefore been pointed out, the invention contemplates introducing the gases which pass into the retort 10 either by means of a tuyère, or, by merely opening the bottom to allow the gas to be drawn in. Accordingly, in such modification of operation which is characterized 35 by the introduction of gas through an open bottom, the use of the tuyères may be wholly or partially discontinued and all or a part of the gas introduced or admitted through the open bottom. In one method of operating with an open 40 bottom, the sealing liquid in the seal 35 may be removed and the primary gas will then have free entrance to the lower extension of the retort. However, the sealing apparatus may be wholly dispensed with and the lower portion of the retort 45 left open to admit air or other gas as conditions of operation may dictate.

It will be noted that in the apparatus of Fig. 1, all of the secondary and tertiary air is supplied by the blower or air compressor 22. By 50 filtering or otherwise appropriately cleaning the air supplied to the blower or compressor, contamination of the zinc oxide product by such substances as dust, soot and the like ordinarily suspended in the atmosphere around a zinc oxide plant may be effectively prevented.

In the apparatus shown in Fig. 2 of the drawing, the suction of the fan 25 is utilized for drawing into the flue system both the secondary and tertiary air in controlled amount. The zinc vapor

issuing from the outlet 17 (of the off-take pipe 14) is oxidized or burned by air drawn into the lower end of the flue 24 through adjustable openings 28. A slide damper 29 is operatively associated with each opening 28 for adjusting the 5 effective area of the opening. Tertiary air is admitted through openings 30 provided with adjustable slide dampers 31. In accordance with the invention, either or both of the series of openings 28 and 30 is regulated and controlled, with 10 respect to the effective area thereof, in such manner as to control the suction thereby applied to the retort.

The gases introduced into the bottom of the retort may be air, reducing gases (e. g., water 15 gas), steam, nitrogen, carbon dioxide, etc.

We claim:

1. The method of making zinc oxide which comprises heating an elongated upright porous column of mixed and agglomerated zinciferous and carbonaceous materials through a wall to produce zinc vapor, introducing gas into said column near its base to facilitate the passage of zinc vapor upwardly therethrough, withdrawing a gaseous stream containing zinc vapor from the 25 upper end portion of the column, introducing a blast of oxidizing gas into the stream to produce zinc oxide, pneumatically transporting the resulting zinc oxide through a conduit to a collecting zone and collecting zinc oxide therein, and introducing a controlled amount of air into said conduit 30 to facilitate the transport of zinc oxide therethrough and simultaneously to regulate the amount of gas introduced into the base of the column. 35

2. The method of making zinc oxide which comprises heating an elongated upright porous column of mixed and agglomerated zinciferous and carbonaceous materials through a wall to produce zinc vapor, introducing gas into said column near 40 its base to facilitate the passage of zinc vapor upwardly therethrough, withdrawing a gaseous stream containing zinc vapor from the upper end portion of the column, introducing a blast of oxidizing gas into the stream to produce zinc 45 oxide, pneumatically transporting the resulting zinc oxide through a conduit to a collecting zone and collecting zinc oxide therein, introducing a controlled amount of air into said conduit to facilitate the transport of zinc oxide there- 50 through and simultaneously to regulate the amount of gas introduced into the base of the column, and regulating the amount of oxidizing gas introduced into the stream of zinc vapor to regulate the amount of gas introduced into the 55 base of the column.

EARL H. BUNCE.  
 HARRY M. HASLAM.